

## UNITED STATES PATENT OFFICE

2,451,148

## PROCESS OF SPINNING VISCOSE ARTIFICIAL SILK, FILAMENTS COMPRISING THREADS, STAPLE FIBERS, BANDS, AND THE LIKE

Theeuwes Albertus Hendrikus Blaas, deceased, late of Nimeguen, Netherlands, by Johanna Geertrui Blaas, nee Westendorp, widow, Epse, Gorssel, Netherlands, assignor to Naamlooze Venootschap Kunstzijdespinnerij Nyma, Nimeguen, Netherlands

No Drawing. Application January 30, 1946,  
Serial No. 644,440  
In the Netherlands June 29, 1943

8 Claims. (Cl. 18—54)

1

The invention relates to an improvement in the process of spinning viscose artificial silk, filaments comprising threads, staple fibres, bands and the like and especially to a method for preventing the obstruction of the spinning nozzles, which is caused by the slow clogging of the orifices during spinning. The said obstruction is especially serious when using a spinning bath containing zinc sulphate.

It has repeatedly been attempted to meet the said difficulty by the addition to the spinning bath of surface-active substances. The addition has been proposed to the spinning bath and/or to the viscose of compounds with a surface-active anion and also of compounds with a surface-active cation. The addition of a compound with a surface-active anion does not bring about an appreciable improvement. A drawback of the addition of compounds with a surface-active cation is that the presence of these compounds in the spinning bath, where they accumulate either by direct addition thereto or, when added to the viscose, during spinning, causes strong foam formation when the spinning bath is regenerated, viz in the concentration thereof by evaporation. Another drawback is that the alkyl pyridinium salts which represent the best accessible class of these compounds are rapidly decomposed in the alkaline viscose so that they can only be used as an addition to the spinning bath.

It is an object of the invention to provide a method which ensures regular spinning without obstruction of the nozzles. Another object of the invention is the addition of compounds which are stable in acid as well as in alkaline liquids. Still another object is not to use additions causing foam formation in concentrating the spinning bath by evaporation.

According to the invention small amounts of certain compounds or salts of compounds are added to the spinning bath or to the spinning solution or if desired to both, which do not reduce the surface-tension of aqueous solutions and are thus not surface active.

The substances which are suitable for addition have the following structure-formula:



2

wherein R represents an aromatic radical containing no more than 6 carbon atoms, R' represents a substituent selected from a class consisting of hydrogen, aliphatic hydrocarbon groups containing no more than 2 carbon atoms and aryl groups containing no more than 6 carbon atoms, and X represents a substituent selected from a group consisting of OH and a monovalent acid radical. Furthermore the pyridinium nucleus can 5 be replaced by a homolog or derivative of pyridinium. The compounds in view can according to F. Kröhnke, Ber. 67, 656 (1934); 68, 1351 (1935) be prepared from pyridinium or a homolog or derivative of pyridinium, an alkali halide which 10 may or may not be substituted and an aldehyde. Pyridinium halides or other pyridinium salts with a monovalent acid radical or compounds from which such pyridinium salts can be formed under the reaction circumstances can also be used as 15 a starting material. Furthermore the compounds to be used according to the invention can also be prepared from other starting materials, e. g. from styrene, bromohydride or from homologs or derivatives of pyridinium.

20 The indicated compounds are generally speaking not only stable in diluted acids, but also in cold diluted alkaline liquids and they can therefore be added to the viscose as well as to the spinning bath. The compounds not being surface-active 25 30 there is no foam formation when concentrating the spinning bath in the regeneration thereof.

From the following examples elucidating the invention the beneficial effect of the addition will become evident.

35 *Example I*

N( $\alpha$ -furyl-2' hydroxy-2' phenyl-1' ethyl)-1 pyridiniumbromide. An equivalent amount of furfural is added to a solution of benzylpyridiniumbromide in ethanol. After the addition of 10 n. sodium lye the reaction mixture is deposited during 5 days at 0° C. The separated product is washed with alcohol and treated with decolorizing carbon and then recrystallized from water of 40 45 70° C. The product melts at 207° C. under decomposition.

0.1% of this compound was dissolved in a spinning bath containing in addition to normal quantities of sodium sulphate and sulphuric acid, 50 g. 50 of zinc sulphate per litre. After spinning for about 1 hour microscopical examination proved that 80% of the orifices was completely clear, whereas in spinning under the same circumstances

but without addition 0% of the orifices proved to be clear.

*Example II*

N( $\alpha$ -furyl-2' hydroxy-2' vinyl-1' ethyl)-1 pyridiniumbromide.

This compound is prepared from furfural and allylpyridiniumbromide. The melting point is not sharply defined. The decomposition begins at 140° C.

0.1% of this compound was dissolved in a spinning bath containing in addition to the normal amounts of sodium sulphate and sulphuric acid 50 g. of zinc sulphate per litre. After spinning for about 8 hours the obstruction of the orifices in the nozzles used was trifling as compared with the obstruction in nozzles used without this addition.

*Example III*

N(phenyl-2' hydroxy-2' ethyl)-1 pyridinium-methosulphate was prepared from methylpyridiniummethosulphate, containing the group  $\text{SO}_4\text{CH}_3$  and benzaldehyde. 0.1% of the reaction product was added to a spinning bath with normal amounts of sodium sulphate and sulphuric acid and 50 g. of zinc sulphate per litre.

After spinning for about 1 hour still over 60% of the orifices was completely clear, whereas microscopical examination of the nozzles after spinning in a bath of the same composition but without addition proved that only 10% of the orifices was still clear.

*Example IV*

N(phenyl-2' hydroxy-2' vinyl-1' ethyl)-1 pyridiniumbromide was prepared from allylpyridiniumbromide and benzaldehyde. 0.1% of this compound was added to viscose and spinning took place in a bath with normal amounts of sodium sulphate and sulphuric acid and 50 g. of zinc sulphate per litre.

After spinning for about 1 hour microscopical examination proved that over 80% of the orifices was still completely clear. In checking the nozzles after spinning in a bath of the same composition but without addition 0% of the orifices appeared to be clear after the same duration of spinning.

*Example V*

N(phenyl-2' hydroxy-2' vinyl-1' ethyl)-1 pyridiniumchloride was prepared from allylpyridiniumchloride and benzaldehyde.

0.1% of this compound was dissolved in a spinning bath as described above. After spinning during 8 hours microscopical examination proved that still over 90% of the orifices was completely clear, whereas only 10% of the orifices in the nozzles used in comparative tests, wherein the same viscose was spun in the same bath, without addition however, did not show obstruction.

*Example VI*

0.07% of N(phenyl-2' hydroxy-2' vinyl-1' ethyl)-1 pyridiniumchloride is added to viscose and the viscose is extruded into a bath with normal sodium sulphate and sulphuric acid content and 50 g. of zinc sulphate per litre.

After spinning during about  $\frac{3}{4}$  of an hour microscopical examination proves that still 95% of the orifices is completely clear, whereas in nozzles used for spinning of a normal viscose in a spinning bath of the same composition only about 10% of the orifices was still clear.

The structural formulae of the compounds of Examples I to VI are:

*Example I*



*Example II*



*Example III*



*Example IV*



*Example V*



*Example VI*



It will be understood that the invention is not limited to the compounds, amounts added, spinning baths used or other data given by way of examples in the above modes of proceeding.

Having thus described the invention what is desired to secure by Letters Patent and claimed:

1. In the spinning of viscose, employing spinning nozzles which tend to become clogged, the process which comprises preventing such clogging by adding to at least one of the liquids which come into contact with said nozzles during spinning a small amount of a pyridin compound which is not surface active of the general formula:



## 5

wherein R represents an aromatic radical containing no more than 6 carbon atoms, R' represents a substituent selected from a class consisting of hydrogen, aliphatic hydrocarbon groups containing no more than 2 carbon atoms and aryl groups containing no more than 6 carbon atoms, and X represents a substituent selected from a group consisting of OH and a monovalent acid radical.

2. The process of claim 1 wherein R' represents 10 a vinyl radical.

3. The process of claim 1 wherein R represents phenyl.

4. The process of claim 1 wherein R represents a furyl radical.

5. The process of claim 1 wherein R' represents phenyl.

6. The process of claim 1 wherein the quantity of pyridine compound added is sufficient to produce a concentration of the order of 0.1 per cent by weight.

7. Process for producing artificial filaments, threads, fibres, staple fibres and the like from viscose, comprising the addition, in any stage of the process, to at least one of the liquids coming into contact with the nozzles during spinning of 0.1% of N( $\alpha$ -furyl-2'-hydroxy-2' vinyl-1' ethyl)-1 pyridiniumbromide,



## 6

8. Process for producing artificial filaments, threads, fibres, staple fibres and the like from viscose, comprising the addition in any stage of the process, to at least one of the liquids coming into contact with the nozzles during spinning, of 5 0.1% of N(phenyl-2'-hydroxy-2' vinyl-1' ethyl)-1 pyridiniumchloride,



15 JOHANNA GEERTRUI BLAAS

NÉE WESTENDORP,

Personal representative authorized to file patent applications on behalf of Theeuwes Albertus Hendrikus Blaas, Deceased.

20

## REFERENCES CITED

The following references are of record in the file of this patent:

## UNITED STATES PATENTS

| Number    | Name  | Date          |
|-----------|-------|---------------|
| 2,125,031 | Polak | July 26, 1938 |

## FOREIGN PATENTS

| 30 Number | Country | Date          |
|-----------|---------|---------------|
| 641,270   | Germany | Jan. 26, 1937 |
| 641,271   | Germany | Jan. 26, 1937 |

35